

Dec. 15, 1942.

J. J. HOPFIELD

2,305,246

MIRROR

Filed June 19, 1939



Fig. 1.



Fig. 2.



Fig. 3.



Fig. 4.

Inventor  
JAMES J. HOPFIELD.

By

Green Green,  
Attorney

## UNITED STATES PATENT OFFICE

2,305,346

## MIRROR

John J. Hopfield, Toledo, Ohio, assignor to  
 Libbey-Owens-Ford Glass Company, Toledo,  
 Ohio, a corporation of Ohio

Application June 19, 1939, Serial No. 279,792

4 Claims. (CL 117—35)

This invention relates to mirrors in general and more particularly to the manufacture of glass mirrors having metallic reflecting coatings.

One known method of making mirrors of this type is to apply molten aluminum to one surface of a glass sheet or plate by spraying the same thereon with a metallizing gun. The present invention contemplates the provision of a novel method of producing mirrors of this type whereby the quality of the mirror and the specular reflection of the sprayed aluminum or other metallic coating is greatly improved. Briefly, this is accomplished by subjecting the metallic coating, after it has been applied to the glass, to a relatively high pressure. This can be done in a number of different ways as will be more clearly hereinafter set forth.

I have discovered that by subjecting the metallic coating to a pressure sufficient to induce a flowing of the metal, a much more brilliant coat of metal is provided in contact with the glass surface. This results in a much sharper specular reflection. I have further found that the use of pressure in this manner results in a mirror exceedingly stable to weathering and that the metallic coating requires no additional treatment for the protection thereof, such as does the common mirror backing. Mirrors treated in this manner, using aluminum or other metal, are useful for many purposes such as in the home, the rear view mirrors of automobiles, and decorative and outdoor mirrors of all kinds.

In the drawing, wherein like numerals are employed to designate like parts throughout the same:

Fig. 1 is a perspective diagrammatic view showing the spraying of the metal coat upon one surface of a glass sheet; and

Figs. 2, 3, and 4 are diagrammatic views illustrating three different ways in which the pressure may be applied to the metal coat.

With reference to the drawing, there is illustrated in Fig. 1 the coating of the upper surface of a glass sheet 18 as it is supported horizontally upon the top of a suitable table or the like 11. The numeral 12 designates a metallizing gun of any conventional or preferred construction by means of which molten aluminum 13 is sprayed upon the glass sheet to form a coating 14 of the desired thickness thereon. Although I have referred to the coating 14 as being of aluminum, it will be understood that the better weathering aluminum alloys can also be used and the word "aluminum" as used herein and in the claims is therefore to be understood as also including

suitable aluminum alloys. Likewise, other ductile metals, such as, for example, copper, may be used.

After the metallic coating 14 has been sprayed upon the glass sheet, it is adapted to be subjected to a pressure sufficient to cause a flowing of the metal. This may be done while the metal is still hot or after it is cold. Further, the metal coat may be reheated before the pressure is applied if desired. As shown in Fig. 2, the pressure is applied by laying the metal coated glass sheet 18 upon a suitable support 15 and passing it beneath a rotatable roll 16. Of course, the support 15 may be maintained stationary and the roll 16 moved thereover if preferred.

In Fig. 3, the pressure is applied by passing the metal coated glass sheet 18 between a plurality of pairs of pressing rolls 17 and 18, while, in Fig. 4, the metal coated glass sheet is subjected to pressure between the platens 19 and 20 of a mechanical or hydraulic platen press.

The pressure may be applied under ordinary room conditions, in prepared atmospheres or in a vacuum. Likewise, any temperature up to the melting point of the metal may be used. While the invention is not limited to any particular degree of pressure, the amount of pressure applied should be sufficient to effect the desired flowing of the metal. The words "flow" and "flowing" are used herein to designate a spreading of the metal upon the application of pressure thereto rather than the flowing of metal in a molten condition.

The flowing action of the metal may also be accomplished in other ways, such as by scraping, buffing or burnishing with a suitable tool, wheel, or brush; by machining or spinning action; hammering or bombardment with shot. It may also be desirable with any of the above pressing operations to employ sheets of paper, cloth, leather, resin, or metal or other materials to assist in the flowing of the metal and/or to protect the glass from breakage. Further, lubricants or other materials can be applied to the metal surface to help the process of flow.

I claim:

1. The method of making a glass mirror having a metallic reflecting coating, which comprises spraying a coating of molten ductile metal upon the back surface of a transparent glass sheet or plate, and then subjecting said metallic coating to pressure sufficient to cause a flowing of the metal at the glass-metal interface to increase the specular reflection of the inner surface of the

metal in contact with the glass when viewed through the glass sheet or plate.

2. The method of making a glass mirror having a metallic reflecting coating, which comprises spraying a coating of molten aluminum upon the back surface of a transparent glass sheet or plate, and then increasing the specular reflection of the inner surface of the aluminum coating in contact with the glass when viewed through the glass sheet or plate by subjecting said aluminum coating to pressure sufficient to cause a flowing of the metal at the glass-metal interface.

3. A method of improving the specular reflec-

tion of a mirror comprising a transparent glass sheet or plate having a sprayed coating of ductile metal upon the back surface thereof, including the step of subjecting the metallic coating to pressure sufficient to cause a flowing of the metal at the glass-metal interface.

4. A method of improving the specular reflection of a mirror comprising a transparent glass sheet or plate having a sprayed coating of aluminum upon the back surface thereof, including the step of subjecting the aluminum coating to pressure sufficient to cause the said aluminum to flow at the glass-metal interface.

JOHN J. HOPFIELD.